

W. A. HUSSY.  
ELECTROLYTIC CYANIDING PROCESS.  
APPLICATION FILED APR. 15, 1913. RENEWED APR. 17, 1919.

1,324,352.

Patented Dec. 9, 1919.

2 SHEETS--SHEET 1.



Fig. 1.



Fig. 2.

*WITNESSES:*

*H. C. Giedner  
Genevieve Ball*

INVENTOR,  
W<sup>m</sup> A. Hussey,  
BY Francis M. Wright,  
ATTORNEY.

1,324,352.

W. A. HUSSEY,

ELECTROLYTIC CYANIDING PROCESS.

APPLICATION FILED APR. 15, 1913. RENEWED APR. 17, 1919.

Patented Dec. 9, 1919.

2 SHEETS—SHEET 2.



WITNESSES:

*H. C. Giedner*  
*Genevieve Ball*

INVENTOR,  
*Wm A. Hussey,*  
BY *Francis M. Wright.*  
ATTORNEY

# UNITED STATES PATENT OFFICE.

WILLIAM A. HUSSEY, OF OAKLAND, CALIFORNIA, ASSIGNOR, BY MESNE ASSIGNMENTS, OF THREE-FOURTHS TO JAMES H. ALLING AND ONE-FOURTH TO FRANCIS M. WRIGHT, BOTH OF SAN FRANCISCO, CALIFORNIA.

## ELECTROLYTIC CYANIDING PROCESS.

1,324,352.

Specification of Letters Patent.

Patented Dec. 9, 1919.

Original application filed June 26, 1912, Serial No. 705,947. Divided and this application filed April 15, 1913, Serial No. 761,246. Renewed April 17, 1919. Serial No. 291,964.

To all whom it may concern:

Be it known that I, WILLIAM A. HUSSEY, a citizen of the United States, residing at Oakland, in the county of Alameda and 5 State of California, have invented new and useful Improvements in Electrolytic Cyanid Process, of which the following is a specification.

The present invention relates to an 10 proved method of recovering precious metals from pulverized ores containing the same, and is a division of an application filed June 26, 1912, Serial Number 705,947, the object of the invention being to provide 15 such a method by which said recovery may be more complete than heretofore, effected in much less time, and at a low cost, and with which the operation can be carried on continuously without interruptions except 20 only for the removal of the recovered metals and then at only long intervals of time.

In the accompanying drawings, Figure 1 is a broken vertical longitudinal section of 25 an apparatus for carrying out my improved process; Fig. 2 is a similar view of another form thereof; and Fig. 3 is a diagrammatic view of two electrolytic machines by which my improved process is carried out.

30 Referring to the drawing, 1 indicates the main body of an apparatus for practising my improved process, composed of insulating material, such as vulcanized rubber, the upper surface of which is formed with a longitudinal series of recesses or depressions 35 2 forming electrolytic cells, and which is arranged at any suitable inclination. Said apparatus is more fully described in the parent application hereinbefore referred to.

40 The height of the upper end of the apparatus is considerably greater than that of the lower end, so that each cell is at a corresponding depth below the preceding cell and at a corresponding height above the 45 next succeeding cell.

In the bottom of each cell 2, at the upper end thereof, is secured, by a suitable conducting bolt 9, a transverse cathode bar 11 of any suitable metallic material. 12 indicates a cover which fits closely upon the upper raised edges of the sides 13 of the body of the apparatus and entirely excludes the

light from the interior thereof and prevents the escape of gases directly upward, their longitudinal escape being prevented when 55 the apparatus is in operation by the water flowing into and out of the apparatus, and secured to said cover 12 between said sides 13 are holders 14 of any suitable insulating material arranged in longitudinal series, one 60 above each of the said cells 2.

In the form of the apparatus shown in Fig. 1, there is secured in a recess in the lower end of each holder, an anode 15, preferably of graphite or other suitable material, 65 and in a recess in the upper portion of each holder a pole 16, also of graphite or other suitable material. Each cell is, as shown at 17, filled with mercury to a suitable depth. All the anodes 15 are electrically connected 70 by wires 18, and a wire 10, to the positive pole of an electric generator, and all the cathode plates or bars 11 are also electrically connected by means of their bolts 9, and a wire 19, to the negative pole of said machine. A wire 20 electrically connects each pole 16 outside the apparatus with the corresponding bar 11. 75

I shall first explain the nature of the process employed in the form of apparatus shown 80 in Fig. 1, before describing the second form thereof.

In this process the pulp to be treated, mixed with a certain proportion of sodium cyanid solution is fed into the apparatus, 85 the electric generator being supposed in operation. On arriving at the first cell and being subjected to electrolysis, sodium cyanid is decomposed, nascent cyanogen being liberated at the anode, and sodium being 90 deposited on the mercury cathode, and probably forming therewith sodium amalgam. It is found that the mercury and sodium at the surface are, by the force of the electric current, on account of the anode being located at the discharge end of the cell and the cathode, in the intake end thereof, driven in a direction against the flow of the pulp into the intake part of the cell, out of the region of electrolysis. The sodium decomposes the water to form caustic soda, and 100 nascent hydrogen is given off, the nascent cyanogen in the presence of alkali dissolves the fine particles of gold, and the caustic

soda immediately decomposes any organic or greasy particles upon the gold and renders it bright and readily amalgamable by the sodium amalgam.

- 5 It is found that the intake portion of the recess, where this chemical reaction takes place, forms in effect a voltaic cell, generating electricity, which, unless the circuit be completed through said cell, would render 10 the pole 16 polarized, and thus generate a counter electro-motive force, and which would thus prevent any further above-described action of said voltaic cell. It is for this reason that I connect each electrode 16 15 with the corresponding bar 9 by a conductor 20 outside of the cell, so that the current generated may be conducted away and the counter electro-motive force be no longer developed. It is found that said current thus 20 generated has a difference of potential of about two volts. Each cell is thus composed of an electrolytic region, in which electrolysis takes place, and a voltaic region, in which chemical reactions occur tending to restore 25 to its former condition the electrolyte flowing through the apparatus, and thus completing the cycle of chemical action, at the same time generating low voltage electric current.
- 30 It is to be noted that in the apparatus shown in Fig. 1 this chemical action can only take place when the mercury and sodium flow out of the electrolytic region. In my second form of apparatus, shown in Fig. 35 2, I do not depend entirely upon the flow of the mercury in the cell to cause its removal out of the electrolytic region, but I also move the electrolytic region itself. In this form of the apparatus, instead of there being a 40 single anode 15 and a single pole 16, as shown in the first form of the invention, there are, for each cell, a large number of electrodes or poles, each of which is used in succession as an anode of an electrolytic cell, 45 the remainder being then used as poles of voltaic cells. These electrodes or poles are shown at 21, and corresponding ones, or those in like order, in all the cells are connected by wires 22 to a common contact 23 50 in a terminal block 24. These contacts 23 are individually connected by wires 26 to spring contacts 27 which normally rest in contact with conductors 28 connected to a wire 29 which is connected by a wire 31 to the negative pole of an electric generator 33 and also 55 by wires 32 to the several cathode bars 11. From the positive pole of said generator a wire 34 leads by a wire 35 and individual wires 36 to contacts 37. Said spring contacts 27 carry rollers 38 which are arranged adjacent to the circumference of a cam roller or timer 39, having a raised portion 41. Said timer is rotated at any suitable speed, so that said raised portion 41 contacts with 60 each roller in succession and then raises the 65

roller so that the spring contact 27 moves out of contact with the conductor 28 and into contact with the contact 37. The slope of this raised portion is such that, just before each spring contact 27 moves out of contact 70 with its corresponding contact 37, the next spring contact 27 of the series moves into contact with its contact 37, so that there is no interruption of the current flowing from the electric generator. 75

It will be seen that, with this construction, each electrode 21 in succession is included in the circuit through the generator, so that the electric current generated thereby can pass through said electrode and through the pulp 80 to the mercury cathode and then to the cathode bar and back to the generator, and the other electrodes are connected directly with the cathode bars 11 outside the apparatus and thus serve as poles of voltaic cells. 85 In other words, the mode of operation of this form of apparatus is electrically similar to that of the first form, except that the position of that electrode which is in actual operation is constantly shifting. The parts 90 are so arranged, that, first, the current from the generator passes through the lowermost electrode 21 the others being short-circuited through the cathode, then through the next higher electrode, and so on up to the uppermost electrode. While the current from the generator is passing through any one electrode sodium cyanid is decomposed by electrolysis beneath said electrode, sodium is deposited upon the mercury cathode immediately beneath said electrode, and, upon the remaining surface of the mercury cathode, the reverse or regenerating process is taking place, that is, the sodium decomposes the water to form caustic soda, and nascent hydrogen is given off. The process applied to each portion of the pulp is that, first, that electrolytic current is passed through the pulp, with the result before explained, and then this electrolytic current is arrested for a 100 period of time longer than the passage of the current and the chemical and voltaic action before described then takes place. All of the pulp is undergoing this process, although the different portions of the pulp are not similarly acted upon at the same time. One small portion, say one-fifth, of the cell is 105 electrolytic, and the remaining portion is voltaic. 110

It will thus be seen that in this apparatus 115 not only is the entire mass of pulp moved over the whole of the cathode, but also the effect produced is the same as if the anode were moved over the whole of the cathode.

It is well known that, in the treatment of 120 gold and silver bearing tellurid, arsenical, antimonial, as well as pyritic ores generally, ordinary cyanid solutions, that is, solutions to which other reagents have not been added, have up to the present time only yielded a 125 130

partial gold and silver extraction, this result being due to the insolubility, and also to the reducing action, of the minerals incasing the gold or elements, as tellurium, combined with it. The addition of cyanogen bromid or iodid to the cyanid solution is found to greatly aid and improve the gold extraction; but the difficulty of preparing these reagents, together with their instability, and 10 the excessive cost involved, has, in most cases, made their application useless or prohibitive. It has also been found that these halogen cyanids are entirely consumed at each application, and no means up to the 15 present time have been known for the repeated and economical regeneration of these special reagents, so as to permit of the economical cyanidizing of ores of the character referred to.

20 Now in the employment of my improved process for such rebellious ores, the ore, having been first crushed to a pulp, is discharged into the top of the apparatus with a certain percentage of sodium cyanid solution containing a haloid alkaline salt, such as sodium bromid. When passing between the anodes 15 and the cathodes 11, by the action of the electric current, electrolysis takes place of a certain portion both of the 25 sodium cyanid and sodium bromid, which thereupon give up their sodium to the mercury and incidentally produce cyanogen bromid, which has the valuable effect before referred to in improving the gold extraction, as the cyanogen bromid powerfully attacks a part of the gold, forming a gold 30 cyanid or bromid, which readily dissolves in the remaining sodium cyanid solution present in the electrolyte.

35 Now upon passing out of the influence of the electrolytic current, the sodium decomposes water and caustic soda and nascent hydrogen are produced. The caustic soda and nascent hydrogen produce the very valuable result that they then reduce the free 40 cyanogen bromid again to sodium cyanid and sodium bromid, while the gold is contained in an aurous cyanid solution. Any gold that is not precipitated from the cyanid 45 solution by electrolysis in the apparatus can be recovered by ordinary methods such as the use of zinc dust, or preferably by the use of zinc anodes, as hereinafter more fully explained.

50 The value of the invention consists in that, whereas the powerful cyanogen bromid is very unstable, by this method any excess of unused cyanogen bromid is, until again needed, immediately converted into the 55 stable compounds sodium cyanid and sodium bromid.

The following chemical reactions occur:

1.  $\text{NaCn} + \text{NaBr}$ , employing a mercury cathode, gives, with the direct electrolytic current, sodium, and  $\text{CnBr}$  (cyanogen bro-

mid) or other halogen cyanid according to the salt applied.

2. On being free from electrolysis, the sodium forms with water, sodium hydrate ( $\text{NaHO}$ ), and nascent hydrogen.

3. These reagents reduce the cyanogen bromid according to the following equation:



The original reagents applied are thus regenerated.

By this method there is substantially no loss of the cyanogen compounds, as, after having served their purpose in the electrolytic apparatus, they can be pumped back and used over again therein.

In the practical application of my improved process it is desirable for economy and other reasons to use two electrolytic machines or apparatus. In the first, A, of such machines there are used graphitized or other insoluble anodes 15<sup>a</sup>, and in the second machine, B, there are used soluble anodes 15<sup>b</sup>, as zinc. In the first or upper machine, A, 90 the main electro-chemical action takes place, while the lower machine B is used for the purpose of obtaining a further or more complete electro-deposition or precipitation of the gold contained in the electrolyte.

The lower machine has soluble zinc anodes instead of insoluble graphitized carbon anodes for the following reason: The sodium cyanid electrolyte is employed, as has already been explained, for two purposes. First, to render the larger particles of gold readily amalgamable by mercury, and, second, to dissolve the finer particles of gold, and form a soluble cyanid of gold and sodium. For the electrolytic recovery of gold 105 from such solution of cyanid of gold and sodium, anodes might be used, as previously stated, which are insoluble, as graphitized carbon, but it is preferable to use soluble anodes as zinc, the chemical affinity of which 110 with cyanogen is very strong.

One advantage gained by using graphitized or other insoluble anodes in the primary electrolytic machine, instead of soluble or zinc anodes, is that the amalgam obtained 115 in the mercury cathode cells where insoluble or graphitized carbon anodes are employed is a pure gold amalgam, free from zinc.

Therefore the difficulty is avoided of separating the gold from the zinc entering the 120 mercury of the mercury cathode through the soluble zinc anodes. Also the insoluble or graphitized carbon anodes are necessary in the first or primary machine, because in this machine the nascent cyanogen is of distinct value for dissolving this fine, or non-amalgamable, gold. In the second or lower machine, in which the larger portion of the dissolved gold is deposited, the acid radicals formed at the anodes are no longer 130

needed, and are highly detrimental to the thorough electro-deposition and saving of the gold.

In the second or lower machine, for the purpose of breaking up the double salts of the gold and sodium cyanid ( $\text{AuNa}(\text{Cn})_2$  or  $\text{AuNa}(\text{Cn})_4$ ), I use at stated intervals a salt, as the sulfate of zinc, the addition being made in minute quantity in solution. This, by destroying the sodium cyanid in the electrolyte, allows of the instant electrode deposition of all gold still present in minute size in the solution.

The following statement will better explain the reaction involved.

The solution of zinc sulfate added to the gold-sodium cyanid solution in the secondary, or soluble zinc-anode machine slowly forms zinc cyanid, aurous cyanid, plus sodium sulfate. The aurous cyanid and zinc cyanid, held in solution momentarily as colloids, are decomposed by electrolysis with the zinc anode, finally forming metallic gold, which is electro-deposited or precipitated in the mercury, and metallic zinc which also is electro-deposited. There probably also form the zinc-sodium cyanids which are washed away in the machine by the current of water continually flowing. The gold in the secondary or soluble (zinc) anode machine is present in solution as already noted, as gold-sodium cyanid. The solution of zinc sulfate, being slowly added to the cyanid electrolyte, breaks up this compound. The zinc, displacing the sodium, unites to form zinc gold cyanid,  $\text{AuZn}(\text{Cn})_2$ , while the  $\text{SO}_4$  ions liberated from the zinc sulfate go over to the sodium to form sodium sulfate. This, while chemically inert in this instance, nevertheless greatly aids in the conductivity of the electrolyte. Gold-zinc cyanid, being colloidal in minute amount in solution, nevertheless remains dissolved sufficiently long to instantaneously effect a complete electro-deposition or precipitation on to the mercury of the gold held in the electrolyte, this being accomplished by means of the soluble zinc anodes employed, and during the continuous flow of the current.

In order to obtain complete extraction and precipitation of the gold from the ore without using a very large number of such machines or apparatus, the pulp is taken from the tail of the first machine and is passed through an agitator 43<sup>a</sup> by means of a centrifugal pump 44<sup>a</sup> and is then delivered to the head of said machine to be again treated therein. This operation is repeated as many times as is necessary to obtain a thorough extraction of the precious values. After this extraction has been accomplished, the pulp is then passed on to the second machine, through which in like manner it is

passed through an agitator 43<sup>b</sup> a number 65 of times in succession by means of a centrifugal pump 44<sup>b</sup>, being agitated between each passage in the manner above referred to, until a thorough precipitation has been effected.

In the claims, for the purpose of brevity, wherever the word sodium is used, it is understood that potassium or other suitable alkaline metal or radical is to be regarded as an equivalent.

I claim:—

1. The method of recovering metal from metalliferous pulp which consists in mixing it with a compound solution of sodium cyanid with a halogen sodium compound, electrolyzing the solution in the presence of a mercury cathode, with a current of sufficient intensity, to form a halogen-cyanogen compound and sodium, and then removing the sodium from the action of the current. 80

2. The method of recovering metal from metalliferous pulp which consists in mixing it with a compound solution of sodium cyanid with a halogen sodium compound, electrolyzing the solution in the presence of a mercury cathode, to form sodium and a halogen cyanogen compound and dissolving the metal by a portion of the compound, forming, by means of the sodium, caustic soda and hydrogen, and transforming the 90 unused compound, by means of the caustic soda and hydrogen, into the original sodium compounds. 95

3. The method of recovering metal from metalliferous pulp which consists in mixing 100 it with a solution of a cyanid with a halogen salt, converting the solution into a halogen-cyanogen compound and a base, employing said compound to dissolve the metal in the pulp, employing said base to restore the 105 unused compound to the original solution, and repeating the above steps in the same order.

4. The process of regenerating a spent 110 cyanid which consists in electrolyzing a sodium compound solution in the presence of a mercury cathode, to produce sodium, employing the sodium to decompose the water of the solution, thus forming nascent hydrogen, and employing the hydrogen to reduce the cyanid compound to a cyanid. 115

5. In the electro-cyanidation of refractory gold and silver ores, the process which consists in first forming a solution of sodium cyanid and a haloid salt, decomposing the solution by electrolysis with a mercury cathode to form a cyanogen haloid compound around the anode and sodium amalgam at the cathode, then interrupting the passage of the current therethrough to permit sodium of the sodium amalgam to decompose water and produce caustic soda and nascent hydrogen, and then intermingling 125

anodic with cathodic products of decomposition to regenerate the original cyanid-bromid solution.

6. In the electro-cyanidation of gold and silver ores, the process which consists in subjecting a compound solution of a cyanid and a haloid salt to electrolysis, thereby forming a cyanogen haloid salt around the anode and sodium amalgam at the mercury 10 cathode of the cell, subjecting the finely pulverized gold and silver ore to the products of electrolysis, for more thorough dissolution of the gold and silver, then interrupting the passage of the current therethrough 15 to decompose the sodium amalgam formed at the cathode, then intermingling anodic and cathodic products of decomposition to regenerate the original solution applied, then adding a zinc salt to break up alkaline

cyanid present in the electrolyte, and finally 20 electro-depositing or precipitating gold and silver dissolved in the electrolyte with soluble anodes as of zinc.

7. The method of precipitating the metal values out of a pulp containing a cyanid 25 electrolyte, which consists in passing an electric current through the mixture in a cell having a mercury cathode and a zinc anode, and adding minute portions of a zinc salt to decompose the alkali cyanids 30 present in the electrolyte.

In testimony whereof I have hereunto set my hand in the presence of two subscribing witnesses.

WILLIAM A. HUSSEY.

Witnesses:

FRANCIS M. WRIGHT,  
D. B. RICHARDS.